

## UNITED STATES PATENT OFFICE

2,479,670

ELECTROPLATING BATHS AND METHOD  
FOR THE ELECTRODEPOSITION OF ZINC

Allan E. Chester, Highland Park, and Frederick F. Reisinger, Waukegan, Ill., assignors to Poor & Company, Chicago, Ill., a corporation of Delaware

No Drawing. Application March 20, 1944,  
Serial No. 527,360

6 Claims. (Cl. 204—55)

1

This invention relates to new and improved cyanide-zinc plating baths, and to a new and improved method for the electrodeposition of zinc.

One of the objects of the invention is to produce new and improved cyanide-zinc plating baths.

A further object is the preparation of new cyanide-zinc electroplating baths useful over a wide range of current densities without burning the electroplated material.

Another object of the invention is to provide new and improved alkaline zinc cyanide electroplating baths which are effective in producing semi-bright, exceptionally smooth zinc plated articles having a pleasing uniform color, while using lower ratios of total sodium cyanide to zinc metal (M ratios) than has heretofore been considered possible for the production of brightening effects in the electrodeposition of zinc.

Another object of the invention is the provision of a new and improved method for the electrodeposition of zinc. Other objects will appear hereinafter.

In the electrodeposition of zinc from alkaline cyanide electrolytes in accordance with the invention, it has now been found that the incorporation of a chromic aldonate into a cyanide-zinc plating bath makes it possible to electrodeposit zinc over a wide range of current densities without burning the plated material. Furthermore, by employing cyanide-zinc plating baths of the type herein described, semi-bright, very smooth zinc plated finishes having a pleasing uniform color are obtained with lower M ratios (ratio of total sodium cyanide to zinc metal) than heretofore used in obtaining brightening effects. Additionally, cyanide-zinc plating baths containing chromic aldonate have enhanced throwing and coloring power.

The term "chromic aldonate" is used herein to describe compounds of trivalent chromium with aldonic acids which may also contain alkali metals, or the like, in their molecules. These compounds are usually prepared in solution form and are preferably made by reacting the solution of the aldonic acid with an alkaline solution of a chromate such as may be prepared, for example, by dissolving chromic anhydride ( $\text{CrO}_3$ ) in water and adding sodium hydroxide. They can also be prepared by reacting the dichromates with an al-

2

donic acid. In our co-pending application Serial No. 527,359, filed of even date herewith, which has matured into United States Patent No. 2,428,356, we describe the chromic aldonates as the product of the reaction of an aqueous alkaline solution of a chromium compound selected from the group of trivalent and hexavalent chromium compounds with an aldonic acid, the ratio of the aldonic acid molecule to the chromium atom being at least 1:1. The chromic aldonate solutions in concentrated form are colored a deep green. When added in relatively small amounts to cyanide-zinc plating baths they impart thereto a brilliant clear green color. These baths are stable and do not tend to precipitate or deteriorate on standing.

The invention will be further illustrated, but is not limited, by the following examples:

*Example I*

20 This example illustrates the preparation of a chromic gluconate. An aqueous solution was prepared by mixing together 1100 grams (11 moles) of chromic acid ( $\text{CrO}_3$ ) and 1650 cc. of water. 900 grams (22.5 moles) of sodium hydroxide were then dissolved in this solution which became warm. This produced an alkaline approximately 21–22% solution of sodium chromate (11 moles). Thereafter, 6000 cc. of 50% gluconic acid (about 15 moles of gluconic acid) containing about 1 to 4% dextrose or other reducing sugars was added with agitation. In 4 or 5 minutes the resultant solution became very hot, with foaming and boiling and the liberation of carbon dioxide. At the end of 35 1 to 2 hours the foam subsided, the product obtained being a very deep green solution. This solution exhibited no precipitation or co-agulation on standing, and may be diluted with water to a beautiful green colored solution. The specific gravity of the concentrated solution was approximately 1.322.

*Example II*

45 A solution was prepared as in Example I, except that 1640 grams of sodium dichromate ( $\text{Na}_2\text{Cr}_2\text{O}_7 \cdot 2\text{H}_2\text{O}$ ) were used instead of the chromic acid and sodium hydroxide. The sodium dichromate was dissolved in 1650 cc. of water and reacted with 6000 cc. of 50% gluconic acid with

agitation. A green colored product was obtained as in Example I, having similar properties.

*Example III*

This example illustrates the preparation of alkaline zinc cyanide electrolytes utilizing chromic gluconates as prepared in Examples I or II.

An electrolyte was prepared by mixing together the following ingredients:

95-100 grams sodium cyanide  
45-55 grams zinc metal (added in the form of zinc oxide)  
100-120 grams sodium hydroxide and enough water to make 1 liter of solution  
2 grams per liter of zinc dust was stirred into the electrolyte, and the entire mixture was filtered in order to remove traces of heavy metals.

This electroplating bath, when employed in a conventional manner, ordinarily produces zinc electroplated articles with a dull gray finish. Upon the addition of either of the products of Examples I or II, however, preferably in amounts corresponding to from 30 to 60 cc. of either of said products per gallon of the above described alkaline zinc cyanide electrolyte, semi-bright, very smooth finishes, having a pleasing, uniform color, were obtained. Furthermore, it was found that the complex aldonate compositions of Examples I or II had a remarkable anti-burn effect, and made it possible to obtain uniform, light gray colored zinc plates over a wide current density range (25-250 amperes per square foot).

One of the important features of the invention is the discovery that with such electrolytes substantial brightening effects are obtained with M ratios within the range of 1.75 to 2.2. The expression "M ratio," as previously indicated, is the ratio of the total weight of sodium cyanide in the bath to the total weight of zinc metal. Heretofore it had been considered that an M ratio of 2.25 to 1 was the lowest M ratio at which brightening effects in zinc plates could be obtained. See "Transactions of American Electrochemical Society," volume 80, page 416 (1941). It is well known that higher M ratios decrease the cathode efficiency. However, by the incorporation of a chromic gluconate into a cyanide zinc electroplating bath, as heretofore described, an M ratio as low as 1.75 to 1 can be used and the cathode efficiency can be increased to 94-96%. At the same time, high current densities, preferably up to 120 amperes per square foot, which is about all that is practical with present commercial installations, can be employed without burning the zinc plated article. By using alternating currents superimposed upon direct currents a good pattern between high current and low current areas can be obtained. Excellent results are obtained with current densities around 70-80 amperes per square foot. As an illustration of the efficiency of the plating operation, at 80 amperes per square foot, it is possible to plate 0.0001" of zinc per minute with a plating bath of the type described in Example III.

The invention is susceptible to some variation and modification in the manner of its practical application. In general, of the chromic aldonates it is preferable to employ a chromic gluconate because the gluconates are the most cheaply and readily available of all of the chromic aldonates. Gluconic acid is ordinarily employed in the preparation of the chromic gluconates in the form of an aqueous solution which usually has a concentration not substantially greater than 50% be-

cause at the higher concentrations it tends to go into the crystalline lactone form. As examples of other aldonic acids which may be used to prepare chromic aldonates, mention is made of the following: mannonic, arabonic, galactonic, and xylonic. The aldonic acids are obtained by the oxidation of the corresponding aldoses and all of them, including gluconic acid, have alpha and beta lactone forms.

- 10 The invention is hereby claimed as follows:
1. An aqueous cyanide-zinc electroplating bath comprising an alkaline cyanide-zinc solution having an M ratio within the range of 1.75 to 2.2 and containing an effective quantity of the product of the reaction of an aqueous alkaline solution of a chromium compound selected from the group consisting of trivalent and hexavalent chromium compounds and an aldonic acid, the ratio of the aldonic acid molecule to the chromium atom in said reaction product being at least 1:1, said product existing in the form of clear green stable solutions in water.
  2. An aqueous cyanide-zinc electroplating bath comprising an alkaline cyanide-zinc solution having an M ratio within the range of 1.75 to 2.2 and containing an effective quantity of the product of the reaction of an aqueous alkaline solution of a chromium compound selected from the group consisting of trivalent and hexavalent chromium compounds and a gluconic acid, the ratio of the gluconic acid molecule to the chromium atom in said reaction product being at least 1:1, said product existing in the form of clear green stable solutions in water.
  3. In a method of electrodepositing zinc the step which comprises electrodepositing the zinc from an alkaline aqueous cyanide-zinc plating bath having an M ratio within the range of 1.75 to 2.2 to which has been added an effective quantity of the product of the reaction of an aqueous alkaline solution of a chromium compound selected from the group consisting of trivalent and hexavalent chromium compounds and an aldonic acid, the ratio of the aldonic acid molecule to the chromium atom in said reaction product being at least 1:1, said product existing in the form of clear green stable solutions in water.
  4. In a method of electrodepositing zinc the step which comprises electrodepositing the zinc from an alkaline aqueous cyanide-zinc plating bath having an M ratio within the range of 1.75 to 2.2 to which has been added an effective quantity of the product of the reaction of an aqueous alkaline solution of a chromium compound selected from the group consisting of trivalent and hexavalent chromium compounds and a gluconic acid, the ratio of the gluconic acid molecule to the chromium atom in said reaction product being at least 1:1, said product existing in the form of clear green stable solutions in water.
  5. A method of electrodepositing zinc which comprises electrodepositing the zinc from an alkaline aqueous cyanide-zinc plating bath having an M ratio within the range of 1.75 to 2.2 to which has been added 30 to 60 cc. per gallon of bath of the product of the reaction of an approximately 50% aqueous solution of gluconic acid containing less than 4% of reducing sugars and an aqueous alkaline solution of a chromium compound selected from the group consisting of trivalent and hexavalent chromium compounds, the ratio of the gluconic acid molecule to the chromium atoms being at least 1:1, said product existing in the form of clear green stable solutions in water, and effecting said electrodeposi-

tion at current densities within the range of 25 to 250 amperes per square foot.

6. An alkaline aqueous zinc-cyanide electroplating bath having an M ratio within the range of 1.75 to 2.2 and comprising about 30 to 60 cc. per gallon of bath of the product of the reaction of an approximately 50% solution of gluconic acid containing about 1 to 4% of reducing sugars with an alkaline approximately 21 to 22% solution of sodium chromate, the relative proportions of sodium chromate to gluconic acid being approximately 11 mols of sodium chromate to 15 mols of gluconic acid, said product existing in the form of clear green stable solutions in water.

ALLAN E. CHESTER. 15  
FREDERICK F. REISINGER.

## REFERENCES CITED

The following references are of record in the file of this patent:

| UNITED STATES PATENTS |           |                |               |
|-----------------------|-----------|----------------|---------------|
|                       | Number    | Name           | Date          |
| 5                     | 694,658   | Meurant        | Mar. 4, 1902  |
|                       | 2,080,520 | Westbrook      | May 18, 1937  |
| 10                    | 2,218,734 | Westbrook      | Oct. 22, 1940 |
|                       | 2,233,500 | Westbrook      | Mar. 4, 1941  |
|                       | 2,406,072 | Gaver          | Aug. 20, 1946 |
|                       | 2,428,356 | Chester et al. | Oct. 7, 1947  |
|                       | 2,443,600 | Chester        | June 22, 1948 |